

# United States Patent Office

3,173,751

Patented Mar. 16, 1965

1

3,173,751

## TEXTILE PROCESS AND COMPOSITION

George C. Daul and Thomas F. Drake, both of Mobile, Ala., assignors, by mesne assignments, to Courtaulds, Limited, London, England, a British company  
No Drawing. Filed Apr. 26, 1961, Ser. No. 105,553  
13 Claims. (Cl. 8—116.4)

This invention relates to a method for improving the properties of cellulose, and in particular to a method for cross-linking cellulose by means of formaldehyde, and to composition for effecting such cross-linking.

For many years it has been known that when cellulose is treated with formaldehyde, various properties, in particular its resistance to swelling by water, are improved. It is considered that such changes occur through cross-linking of the cellulose chains at suitable positions along their length. Although the ability of formaldehyde to cross-link cellulose has been known for perhaps fifty years, no substantial commercial use has been made of this ability, because the processes so far proposed have all had very serious practical drawbacks.

Chiefly such processes have not succeeded because they have used acid catalysts which are difficult to control to avoid excessive tendering of the textile material.

In our copending application Serial No. 81,956, filed January 11, 1961, now Patent No. 3,113,826, we have described the cross-linking of cellulose by means of certain metallic salts which are Lewis acids in the solid state. In the procedure described in said application cellulosic textile material is impregnated with formaldehyde and with high concentrations of the Lewis acid. It is then dried and cured by heating. The process described in our prior application has the distinct advantage over formaldehyde treatments in permitting relatively large amounts of formaldehyde to be chemically combined with the cellulose without objectionable tendering. However, with the specific Lewis acids enumerated in said prior application it is preferred to carry out the process at a pH of 5 or above. Below pH 5, it is found, there is a tendency toward tendering of the cellulose material.

The present invention is based upon the discovery that zinc fluoborate is a good catalyst for the cellulose-formaldehyde reaction. In particular it has been found that cellulose, especially regenerated cellulose textile material, can be cross-linked with formaldehyde using  $Zn(BF_4)_2$  as a catalyst at pH 5 without extensive damage. This is a valuable property, since the use of a low pH in general permits a shorter curing time or a lower curing temperature to be used. Shorter curing times have obvious economic advantages. Lower curing temperatures make it possible to use conventional steam dryers for curing, thus enabling the process to be practiced with equipment which is readily available in many finishing plants.

The invention thus envisions a process for cross-linking cellulose which comprises reacting cellulose with formaldehyde in the presence of zinc fluoborate.

The invention can be applied to any form of cellulose, though it is most useful with regenerated cellulose. Normally the process will find its greatest application in the treatment of filamentary material, though other forms, e.g. paper, board or film may also be treated. The filamentary material may be treated in the form of staple fiber, as continuous filament, or in the form of tow, yarn or thread. The process can also be applied to structures containing cellulose fibers. The structures may be woven or knitted textile fabrics, or textile fabrics of other kinds, for example, the so-called non-woven fabrics, or even paper. The fabrics may be of various constructions; thus they may consist wholly of cellulose fibers or in part of these fibers and in part of fibers of other kinds, for

2

example, cellulose acetate (acetone soluble cellulose acetate or cellulose tri-acetate), or fibers of synthetic linear polymers, for example, of polyamides, such as nylon 6 or nylon 66, or of polyesters, for example polyethylene terephthalate, or of addition polymers derived from acrylonitrile. The cellulose fibers in the fabrics may be staple fibers or continuous filaments. Preferably, when blends are treated, the cellulose fibers comprise at least 35% by weight of the blend.

10 If desired, the cellulose, prior to treating may have been dyed with any of many common dyes, without adverse effect.

The formaldehyde used may be added to the treating solution as the normal 37-40% aqueous commercial solution. Other sources, e.g. paraformaldehyde, may, however, be used as desired.

15 The zinc fluoborate may be added to the treating solution as the anhydrous salt, or as a hydrate. The commercially available solution containing 40%

20  $Zn(BF_4)_2 \cdot 6H_2O$

may also be used.

25 The formaldehyde and the zinc fluoborate are normally applied from aqueous solutions. Other solvents, e.g. methanol or ethanol, may be present without detrimental effect, but the solution should contain at least 10% by weight water. Separate solutions may be used for the formaldehyde and the zinc fluoborate, but no advantage is gained thereby.

30 The concentration of formaldehyde in the treating solution may vary to a considerable extent, depending on whether natural or regenerated cellulose is treated and on the physical form of the fiber. Moreover, where high crease recovery is required, more bound formaldehyde is required in the final product and a higher concentration of formaldehyde is used when the objective is merely a decrease in water imbibition.

35 In general, it is found that the amount of zinc fluoborate deposited on the cellulose is more significant than the concentration of formaldehyde in the solution, provided that enough formaldehyde is present during curing to furnish the quantity of formaldehyde required to be bound to the cellulose for the effect desired. With this in mind, it is found that while solutions containing large concentrations of formaldehyde (say 10 to 20%) and small concentrations of zinc fluoborate (say 0.06 to 0.2%  $Zn(BF_4)_2$ ) may be used, it is preferable to use smaller amounts of formaldehyde, and relatively large amounts of  $Zn(BF_4)_2$ . The use of smaller amounts of formaldehyde is more economical and creates fewer problems in connection with the health and comfort of operators. Moreover, the use of large excesses of formaldehyde increases the tendency toward odor development in the finished product, requiring extensive washing with resultant increased expense.

40 In general, a recommended overall concentration range for formaldehyde would be between about 0.5 and about 6%, and for  $Zn(BF_4)_2$  between about 0.3% and about 3.5%.

45 As noted above one of the advantages of the present invention is that low pH can be used, and preferably the pH of the solution is therefore below about 5, usually between about 1 and about 5, preferably between about 3 and about 5. Above about pH 5, zinc fluoborate hydrolyses to form a precipitate even at low concentrations.

50 The temperature of the treating solution is not especially critical. Room temperature is satisfactory, though lower temperatures may be used to prevent loss of formaldehyde. Normally, temperatures of 15° C. to 50° C. are used.

55 The treating solution may contain various textile auxiliaries such as softening agents, lubricants, water repell-

lants and the like. In general, these materials function in the normal way, i.e. as they would were no formaldehyde present.

The treating solution (or solutions) is applied to the cellulose in such a way that after impregnation and drying the material contains at least 0.2 g. zinc fluoborate,  $Zn(BF_4)_2$ , per 100 g. of cellulose and preferably between about 0.35 and about 4.5 g. per 100 g. of cellulose. Sufficient formaldehyde is picked up so that, bearing in mind losses during drying and curing, between about 0.25 and about 2.5% by weight is chemically bound directly to the cellulose. Formaldehyde is said to be chemically bound if it is not removed by scouring in water for one hour at the boil. It may be determined by measuring the quantity of formaldehyde released upon complete hydrolysis of the treated cellulose with 12 N  $H_2SO_4$ .

As indicated previously, the amount of bound formaldehyde will vary with the effect desired. When fiber is treated as such to reduce water imbibition, 0.25 to say 1.25% by weight bound formaldehyde will be sufficient. To give crease recovery and dimensional stability to textiles 0.5% to 2.5% bound formaldehyde is required.

Normally, for reasons of economy, the weight ratio of zinc fluoborate to formaldehyde deposited on the fiber will be at least 1:20 and preferably between about 1:19 and about 5:1. Larger amounts of formaldehyde may be used, but as explained above this is not desirable.

The actual manipulative steps by which the treating solution is applied will vary with the physical form of the cellulosic material. In the case of staple fiber, a mat or blanket of the material is normally sprayed with the solution followed by a squeezing to remove excess. A continuous filament may be passed through a path or wound on a roller over which the reagent is sprayed. A tow may be laid down in a plaited pattern and sprayed; or passed continuously through a bath. Woven and knitted fabrics may be padded using techniques well known to the art.

In all of these cases, the treatment is preferably carried out so that after removal of excess liquor by squeezing or other means, between say 130% and say 50% of liquor (based on the weight of bone dry unimpregnated material) remains on the material.

Following impregnation, the material is dried at say 30–110° C. for whatever time is required to reduce the moisture content to say 5% or less by weight of the bone dry material and then cured by heating to temperatures from about 110° C. to about 180° C. for periods which may range from say 30 minutes to a few (say about 5) seconds.

The temperature and time for curing must be carefully selected having in mind the pH at which the treatment has been conducted. Thus where a low pH is used, curing may be conducted under mild conditions within the range set forth, with a rather high temperature and a very short time or with a low temperature and a longer time.

Obviously, the drying and curing steps may be combined in a single treatment, if desired.

Following the curing stage, the cellulose may be washed, if desired, with  $NH_3$ , urea or other formaldehyde acceptor to remove unbound formaldehyde and curing agent.

If desired, it may then be subjected to any of a number of conventional after treatments. For example, cellulose fabrics, following treatment by the present process can be mercerized, or sanforized, or both. It is an important advantage of the invention that it permits normal textile trade regenerated cellulose fabrics to be mercerized or sanforized.

As noted above, the product obtained from the present process contains between about 0.25% and about 2.5% formaldehyde chemically bound directly to the cellulose (based on air dry unimpregnated material), as determined by the amount of formaldehyde liberated by complete hydrolysis of the cellulose with 12 N  $H_2SO_4$ .

When the initial material treated in accordance with the invention is regenerated cellulose, the characteristics of the product are quite different from those of the starting material. Thus, although normal regenerated cellulose swells so rapidly in caustic soda that mercerization of regenerated cellulose fabric is not practical, the product of the present invention has a greatly lowered swellability in caustic soda and can be mercerized without difficulty.

Again, regenerated cellulose will dissolve in cuprammonium hydroxide, while the products of the present invention will not. Further, while the water imbibition of conventional textile grade viscose staple fiber is about 100–115%, the water imbibition of the present products can be reduced to around 30–40%.

When cellulose fabrics are treated in accordance with the invention, their dry crease recovery is greatly improved, and is usually increased by at least 50% ( $W+F$ ). In some cases it may be increased by as much as 150% ( $W+F$ ). Moreover, permanent dimensional stability is imparted, even after scouring at acid pH. Since no chlorine retentive groups are introduced into the cellulose, the resistance of fabric treated in accordance with the invention to damage by chlorine bleaches is high.

The invention will be further described with reference to the following specific examples which are given for purpose of illustration only and are not to be taken as in any way limiting the invention beyond the scope of the appended claims.

#### EXAMPLE 1

Fifteen gram samples of never-dried,  $1\frac{1}{2} \times 1\frac{1}{16}$  viscose rayon fiber were soaked for 5 minutes in 100 g. of aqueous solution having a pH of 2.5 and containing 0.3% formaldehyde (from 37% commercial formaldehyde solution) and from 0.3% to 3.0% (by weight) zinc fluoborate hexahydrate. The samples were centrifuged to about 130% pickup of liquid by weight of bone dry cellulose, dried at 80° C. and cured at 155° C. for 6 minutes in a Dietert dryer.

The cured samples were rinsed free of catalyst, dried and conditioned. Dry and wet tenacity determinations were made. Part of each sample was scoured for one hour in water at 95–100° C. and tested for water imbibition value using the procedure described in the Journal of the Society of Dyers and Colourists, October 1948, page 331.

Results are shown in Table A below.

Table A

| HCHO Applied, Percent | $Zn(BF_4)_2 \cdot 6H_2O$ Applied, Percent | G. $Zn(BF_4)_2$ , 100 g. cell. | Denier | Dry Ten., g./d. | Dry Elong., Percent | Wet Ten., g./d. | Water Imbibition, Percent |
|-----------------------|-------------------------------------------|--------------------------------|--------|-----------------|---------------------|-----------------|---------------------------|
| None (Control)        | 0.3                                       | 0.27                           | 1.50   | 2.40            | 22.5                | 1.45            | 98                        |
| 3                     | 0.6                                       | 0.54                           | 1.54   | 2.35            | 14.5                | 1.49            | 62                        |
| 3                     | 1.2                                       | 1.08                           | 1.46   | 2.43            | 12.8                | 1.58            | 48                        |
| 3                     | 1.8                                       | 1.62                           | 1.48   | 2.20            | 9.2                 | 1.56            | 41                        |
| 3                     | 2.4                                       | 2.16                           | 1.52   | 1.90            | 7.0                 | 1.32            | 37                        |
| 3                     | 3.0                                       | 2.70                           | 1.50   | 1.94            | 6.5                 | 1.40            | 36                        |
|                       |                                           |                                | 1.60   | 2.06            | 7.3                 | 1.49            | 39                        |

## EXAMPLE 2

A blanket of freshly spun-never-dried viscose rayon (textile grade) still in the gel state after spinning and having a gel-state water imbibition value of 140% was pre-squeezed between pressure rolls to a liquid retention of about 100% on the weight of cellulose.

The squeezed blanket was then passed under a spray of an aqueous solution containing 1.5% by weight of formaldehyde, 1% by weight of zinc fluoborate hexahydrate (from a 40% commercial solution) and 0.4% of a polyglycol stearate finishing agent. The solution had a pH of 3.5.

The impregnation was carried out in two stages with a pressurized intermediate squeeze and a final heavy squeeze (60 lb./linear inch) to a final liquid retention of about 100% on the weight of cellulose.

The treating bath was re-circulated and replenished by

minutes and in the cure zone 7 minutes. The fiber product had a water imbibition value of 50%, a dry tenacity of 2.3 g./d., and a wet tenacity of 1.6 g./d. A control sample had a water imbibition of 120%, a dry tenacity of 2.5 g./d. and a wet tenacity of 1.3 g./d.

After scouring in water at 100° C. for 1 hour, the water imbibition value was 48%, and the bound formaldehyde content was 0.80%.

10

Samples of a rayon challis were soaked for five minutes in baths containing varying amounts of formaldehyde and zinc fluoborate at pH 3.5, padded to 100% pickup, framed, dried for 10 minutes at 80° C. and cured for five minutes at 150° C. or for 3 minutes at 160° C. After curing the samples were washed to remove excess salts, pressed dry, analysed and tested.

Results are listed in Table B below.

Table B

| Bath Make-Up                                      | Cure Conditions | G. Zn(BF <sub>4</sub> ) <sub>2</sub> ,<br>100 g. cell. | Percent<br>Bound<br>HCHO | Percent<br>Scoured<br>W.I. | Dry<br>CRA <sup>1</sup><br>W+F | Wet<br>CRA <sup>1</sup><br>W+F | Elm. Tear <sup>2</sup> |      | R-Strip Ten. <sup>3</sup> |      |
|---------------------------------------------------|-----------------|--------------------------------------------------------|--------------------------|----------------------------|--------------------------------|--------------------------------|------------------------|------|---------------------------|------|
|                                                   |                 |                                                        |                          |                            |                                |                                | Dry                    | Wet  | Dry                       | Wet  |
| 3.0% HCHO, 1.0% Zn(BF <sub>4</sub> ) <sub>2</sub> | 150° C., 5 min. | 1.0                                                    | 0.36                     | 54.7                       | 201                            | 183                            | 1.9                    | 1.4  | 41.1                      | 18.4 |
| 3.0% HCHO, 2.0% Zn(BF <sub>4</sub> ) <sub>2</sub> | 150° C., 5 min. | 2.0                                                    | 0.80                     | 44.0                       | 214                            | 197                            | 1.2                    | 1.3  | 26.0                      | 15.7 |
| 3.0% HCHO, 3.0% Zn(BF <sub>4</sub> ) <sub>2</sub> | 150° C., 5 min. | 3.0                                                    | 1.15                     | 42.4                       | 226                            | 209                            | 0.9                    | 1.0  | 23.7                      | 13.1 |
| 4.5% HCHO, 1.0% Zn(BF <sub>4</sub> ) <sub>2</sub> | 150° C., 5 min. | 1.0                                                    | 1.0                      | 44.2                       | 207                            | 208                            | 2.4                    | 2.1  | 31.4                      | 19.4 |
| 4.5% HCHO, 2.0% Zn(BF <sub>4</sub> ) <sub>2</sub> | 150° C., 5 min. | 2.0                                                    | 1.1                      | 39.6                       | 223                            | 216                            | 1.9                    | 2.3  | 24.0                      | 24.5 |
| 4.5% HCHO, 3.0% Zn(BF <sub>4</sub> ) <sub>2</sub> | 150° C., 5 min. | 3.0                                                    | 1.7                      | 34.7                       | 241                            | 239                            | 1.7                    | 2.1  | 20.5                      | 14.0 |
| 3.0% HCHO, 1.0% Zn(BF <sub>4</sub> ) <sub>2</sub> | 160° C., 3 min. | 1.0                                                    | 0.37                     | 58.0                       | 203                            | 177                            | 2.4                    | 1.8  | 26.1                      | 15.7 |
| 3.0% HCHO, 2.0% Zn(BF <sub>4</sub> ) <sub>2</sub> | 160° C., 3 min. | 2.0                                                    | 0.97                     | 41.3                       | 222                            | 212                            | 1.5                    | 1.3  | 21.0                      | 13.8 |
| 3.0% HCHO, 3.0% Zn(BF <sub>4</sub> ) <sub>2</sub> | 160° C., 3 min. | 3.0                                                    | 1.08                     | 40.7                       | 217                            | 207                            | 1.6                    | 1.2  | 18.3                      | 9.8  |
| 4.5% HCHO, 1.0% Zn(BF <sub>4</sub> ) <sub>2</sub> | 160° C., 3 min. | 1.0                                                    | 0.93                     | 44.7                       | 200                            | 214                            | 2.1                    | 2.0  | 28.1                      | 18.5 |
| 4.5% HCHO, 2.0% Zn(BF <sub>4</sub> ) <sub>2</sub> | 160° C., 3 min. | 2.0                                                    | 1.3                      | 40.7                       | 229                            | 225                            | 1.7                    | 2.0  | 17.0                      | 16.3 |
| 4.5% HCHO, 3.0% Zn(BF <sub>4</sub> ) <sub>2</sub> | 160° C., 3 min. | 3.0                                                    | 1.9                      | 39.6                       | 246                            | 230                            | 1.6                    | 2.1  | 23.3                      | 13.9 |
| Control Fabric                                    |                 |                                                        | 85                       | 170                        | 160                            | 1.8                            | 1.2                    | 32.2 | 15.6                      |      |

<sup>1</sup> CRA (W+F)=Monsanto Crease Recovery Angle (Warp and Filling); See 1958 Technical Manual, AATCC, p. 157.

<sup>2</sup> Elm. Tear=Elementor Tear Strength; Testing procedure described in ASTM Standards on Textile Materials D1424; p. 607-611.

<sup>3</sup> R-Strip Ten.=Ravel Strip Tensile Strength; Testing procedure described in ASTM Standards on Textile Materials, October 1959, Tests for woven fabrics, D 39, p. 4.

metering in a concentrated mixture of zinc fluoborate and formaldehyde in the correct proportions. Similarly, concentrated finishing agent was added to the bath at a rate

## EXAMPLE 4

The procedure of Example 3 was repeated at pH 5. Results are shown in Table C.

Table C

| Bath Make-Up                                      | Cure Conditions | G. Zn(BF <sub>4</sub> ) <sub>2</sub> ,<br>100 g. cell. | Percent<br>Bound<br>HCHO | Percent<br>Scoured<br>W.I. | Dry<br>CRA <sup>1</sup><br>W+F | Wet<br>CRA <sup>1</sup><br>W+F | Elm. Tear |      | R-Strip Ten. |      |
|---------------------------------------------------|-----------------|--------------------------------------------------------|--------------------------|----------------------------|--------------------------------|--------------------------------|-----------|------|--------------|------|
|                                                   |                 |                                                        |                          |                            |                                |                                | Dry       | Wet  | Dry          | Wet  |
| 3.0% HCHO, 1.0% Zn(BF <sub>4</sub> ) <sub>2</sub> | 150° C., 5 min. | 1.0                                                    | 0.35                     | 63.7                       | 195                            | 174                            | 1.9       | 1.6  | 35.6         | 18.6 |
| 3.0% HCHO, 2.0% Zn(BF <sub>4</sub> ) <sub>2</sub> | 150° C., 5 min. | 2.0                                                    | 0.69                     | 51                         | 203                            | 186                            | 1.5       | 1.4  | 29.7         | 17.9 |
| 3.0% HCHO, 3.0% Zn(BF <sub>4</sub> ) <sub>2</sub> | 150° C., 5 min. | 3.0                                                    | 0.92                     | 44.9                       | 213                            | 193                            | 1.3       | 1.3  | 24.4         | 14.5 |
| 4.5% HCHO, 1.0% Zn(BF <sub>4</sub> ) <sub>2</sub> | 150° C., 5 min. | 1.0                                                    | 0.12                     | 70.0                       | 201                            | 172                            | 2.2       | 1.5  | 34.1         | 17.5 |
| 4.5% HCHO, 2.0% Zn(BF <sub>4</sub> ) <sub>2</sub> | 150° C., 5 min. | 2.0                                                    | 1.0                      | 44.7                       | 216                            | 208                            | 1.4       | 1.3  | 29.4         | 18.4 |
| 4.5% HCHO, 3.0% Zn(BF <sub>4</sub> ) <sub>2</sub> | 150° C., 5 min. | 3.0                                                    | 1.3                      | 40.6                       | 226                            | 214                            | 1.1       | 1.2  | 23.2         | 15.0 |
| 3.0% HCHO, 1.0% Zn(BF <sub>4</sub> ) <sub>2</sub> | 160° C., 3 min. | 1.0                                                    | 0.21                     | 69.5                       | 199                            | 159                            | 2.2       | 1.6  | 36.6         | 19.2 |
| 3.0% HCHO, 2.0% Zn(BF <sub>4</sub> ) <sub>2</sub> | 160° C., 3 min. | 2.0                                                    | 0.62                     | 56.7                       | 216                            | 187                            | 1.5       | 1.4  | 29.9         | 17.9 |
| 3.0% HCHO, 3.0% Zn(BF <sub>4</sub> ) <sub>2</sub> | 160° C., 3 min. | 3.0                                                    | 0.86                     | 45.3                       | 227                            | 197                            | 1.2       | 1.2  | 24.8         | 13.0 |
| 4.5% HCHO, 1.0% Zn(BF <sub>4</sub> ) <sub>2</sub> | 160° C., 3 min. | 1.0                                                    | 0.25                     | 61.2                       | 208                            | 176                            | 1.8       | 1.5  | 30.7         | 15.3 |
| 4.5% HCHO, 2.0% Zn(BF <sub>4</sub> ) <sub>2</sub> | 160° C., 3 min. | 2.0                                                    | 1.1                      | 41.8                       | 230                            | 227                            | 1.1       | 1.2  | 22.6         | 12.2 |
| 4.5% HCHO, 3.0% Zn(BF <sub>4</sub> ) <sub>2</sub> | 160° C., 3 min. | 3.0                                                    | 1.6                      | 35.1                       | 243                            | 218                            | 1.2       | 1.3  | 20.1         | 14.7 |
| Control Fabric                                    |                 |                                                        | 85                       | 170                        | 160                            | 1.8                            | 1.2       | 32.2 | 15.6         |      |

sufficient to maintain the correct concentration in the bath.

The treated, squeezed fiber blanket was opened, laid down as a bed on a conveyor, passed through a drier at a temperature of 105° C. then through a cure zone at a temperature of 160° C. Dwell time in the drier was 20

60

## EXAMPLE 5

The procedure of Examples 3 and 4 was repeated at pH 3.0, with curing at 150° C. for 5 minutes. Results are shown in Table D.

Table D

| HCHO,<br>percent | Bath<br>Zn(BF <sub>4</sub> ) <sub>2</sub> ,<br>percent | G. Zn(BF <sub>4</sub> ) <sub>2</sub> ,<br>100 g. cell. | Bound<br>HCHO,<br>percent | W.I.,<br>percent | Dry CRA<br>W+F <sup>o</sup> | Wet CRA<br>W+F <sup>o</sup> | Grab<br>Tensile,<br>lbs. |
|------------------|--------------------------------------------------------|--------------------------------------------------------|---------------------------|------------------|-----------------------------|-----------------------------|--------------------------|
| 4                | 2                                                      | 2                                                      | 1.0                       | 40               | 239                         | 221                         | 33                       |
| 4.5              | 2                                                      | 2                                                      | 1.6                       | 40               | 238                         | 218                         | 36                       |
| 5                | 2                                                      | 2                                                      | 1.6                       | 38               | 244                         | 219                         | 38                       |
| 4                | 2                                                      | 3                                                      | 1.4                       | 40               | 237                         | 225                         | 29                       |
| 4.5              | 2                                                      | 3                                                      | 1.8                       | 35               | 246                         | 231                         | 37                       |
| 5                | 2                                                      | 3                                                      | 1.8                       | 32               | 246                         | 230                         | 33                       |

7 The control (untreated fabric) and a Crab tensile of about 48 lbs.

EXAMPLE 6

Three samples of the same rayon challis used in Examples 3-5 were treated in a bath containing 4.5% HCHO and 2.0%  $Zn(BF_4)_2$  at pH 2.5. After padding to 100% pickup they were framed to dimension, dried at 80° C. and cured for five minutes at 130° C., 140° C. and 150° C. respectively. After washing and drying they were analysed and tested. The results appear in Table E below.

Table E

| Cure,<br>°C. | Bound<br>HCHO,<br>percent | G. $Zn(BF_4)_2$ ,<br>100 g. cell. | W.I.,<br>percent<br>(scoured) | CRA<br>(W+F)° |     | Grab<br>Ten.,<br>lbs. |
|--------------|---------------------------|-----------------------------------|-------------------------------|---------------|-----|-----------------------|
|              |                           |                                   |                               | Dry           | Wet |                       |
| 130          | 1.4                       | 2                                 | 43                            | 253           | 200 | 37.0                  |
| 140          | 1.2                       | 2                                 | 43                            | 242           | 228 | 44.0                  |
| 150          | 1.6                       | 2                                 | 41                            | 245           | 208 | 39.5                  |

It is thus obvious that with  $Zn(BF_4)_2$  curing can be carried out efficiently at relatively low temperatures.

We claim:

1. A method for cross-linking cellulose which comprises reacting cellulose with formaldehyde in the presence of zinc fluoborate.
2. A method for cross-linking cellulose which comprises impregnating cellulose with zinc fluoborate and with formaldehyde in the presence of water and curing the impregnated cellulose.
3. A method for cross-linking regenerated cellulose filamentary material which comprises impregnating said material with formaldehyde and with an aqueous solution of zinc fluoborate and curing the impregnated material.
4. A method for cross-linking regenerated cellulose filamentary material which comprises impregnating said material with formaldehyde and with zinc fluoborate in the presence of water at a pH not greater than about 5, and curing the impregnated material.
5. A method for cross-linking regenerated cellulose filamentary material which comprises impregnating said material, in the presence of water with formaldehyde and with at least about 0.2 g. per 100 g. of cellulose of zinc fluoborate, and curing the impregnated material.
6. The method claimed in claim 5 wherein the material is impregnated at a pH between about 2 and about 5.

5 7. A method for cross-linking regenerated cellulose filamentary material which comprises impregnating said material with an aqueous solution containing formaldehyde and between about 0.3 and about 3.5% by weight zinc fluoborate and drying and curing the impregnated material.

8 8. A method for cross-linking regenerated cellulose filamentary material which comprises impregnating said material with an aqueous solution containing between 10 about 0.5 and about 6% formaldehyde, between about 0.3% and about 3.5% zinc fluoborate and having a pH between about 2 and about 5 and drying and curing the impregnated material.

9. The method claimed in claim 8 and comprising 15 curing the impregnated material by heating it at between about 100° C. and about 180° C.

10. An aqueous solution for use in cross-linking cellulose comprising formaldehyde and zinc fluoborate.

11. An aqueous solution for use in cross-linking cellulose comprising formaldehyde and at least about 0.3% zinc fluoborate.

12. An aqueous solution for use in cross-linking cellulose comprising between about 0.5% and about 6% formaldehyde, between about 0.3% and about 3.5% zinc 25 fluoborate, and having a pH not greater than about 5.

13. The solution claimed in claim 12 wherein the pH is between about 2 and about 5.

References Cited in the file of this patent

UNITED STATES PATENTS

- 2,311,080 Pinkney ----- Feb. 16, 1943  
2,436,076 Pfeffer ----- Feb. 17, 1948  
2,826,514 Schroeder ----- Mar. 11, 1958  
3,046,079 Reeves, et al. ----- July 24, 1962

FOREIGN PATENTS

- 721,380 Great Britain ----- Jan. 5, 1955

OTHER REFERENCES

40 Schroeder: Textile Research Journal, February 1957, pages 135-145.

Hurwitz et al.: Textile Research Journal, vol. 28, pp. 257-262 (1958).

45 Reinhardt et al.: American Dyestuff Reporter, vol. 47, No. 22, pp. 758-764 (1958).

Guthrie: Textile Research Journal, vol. 33, pp. 995-958, 1963.

UNITED STATES PATENT OFFICE  
CERTIFICATE OF CORRECTION

Patent No. 3,173,751

March 16, 1965

George C. Daul et al.

It is hereby certified that error appears in the above numbered patent requiring correction and that the said Letters Patent should read as corrected below.

Column 1, line 12, for "composition" read -- compositions --; line 47, for "pH.5" read -- pH below 5 --; column 2, line 22, for "fluorborate" read -- fluoborate --; line 36, for "used when" read -- used than when --; column 3, line 33, for "path" read -- bath --; columns 5 and 6, Table B, last column, under "Wet", line 1 thereof, for "18.4" read -- 18.7 --; same column and table, line 2 thereof, for "15.7" read -- 15.4 --; same column and table, line 4 thereof, for "19.4" read -- 19.7 --; column 7, line 1, for "and a Crab" read -- had a Grab --; column 8, lines 47 and 48, strike out "Guthrie: Textile Research Journal, vol. 33, pp. 995-958, 1963.".

Signed and sealed this 14th day of September 1965.

(SEAL)

Attest:

ERNEST W. SWIDER  
Attesting Officer

EDWARD J. BRENNER  
Commissioner of Patents